

# United States Patent Office

3,245,788

Patented Apr. 12, 1966

1

3,245,788

# PRODUCTION OF COLOR PHOTOGRAPHIC IMAGES

Jan Jaeken, Hove-Antwerp, and Robert Leopold Jansseune, Wilrijk-Antwerp, Belgium, assignors to Gevaert Photo-Producten N.V., Mortsel, Belgium, a Belgian company

No Drawing. Filed Apr. 3, 1961, Ser. No. 100,010  
Claims priority, application Great Britain, Apr. 6, 1960,  
12,163/60

12,163/60  
15 Claims. (Cl. 96—9)

The present invention relates to the production of colored photographic images, more particularly to a process of color correction utilizing an integral masking procedure.

procedure. It is known that dyes formed by color development in subtractive multicolor photographic pictures do not transmit all of the light which practical considerations demand. The cyan dye which should absorb red light and transmit green and blue light usually absorbs a small amount of green and blue light, as well as a major proportion of red light. The magenta dye which should absorb green light and transmit blue and red light usually absorbs a considerable amount of blue light and a small amount of red light, as well as a major proportion of green light. The yellow dye which should absorb blue light and transmit green and red light is usually satisfactory.

Due to the above mentioned unwanted side-absorptions of the dyes formed by color development, it is practically impossible to obtain a true reproduction of the original colors on printing multicolor photographic transparencies containing such dyes.

Correction of the colors on printing is therefore desirable, and this is usually done by masking. Since separate masks are difficult to register with the color transparency, it is desirable that the mask be integral with the colored images.

A process for the production of a color photographic image wherein the mask is integral with the colored image is described in U.S. patent applications Ser. No. 705,508, now U.S. Patent 3,012,884, filed December 27, 1957; No. 70,914, now U.S. Patent 3,013,879, filed November 22, 1960, and No. 72,298, now U.S. Patent 3,047,385, filed November 29, 1960, by Maurice Antoine de Ramaix and Jan Jaeken; Ser. No. 66,964, now U.S. Patent 3,079,256, filed November 3, 1960 by Raphael Karel Van Poucke, Arthur Henri de Cat and Marcel Hendrik Verbrugge; and Serial No. 71,117, filed November 14, 1960, by Jozef Frans Willems and Jan Jaeken.

According to said pending applications a color corrected image is formed in a photographic element comprising a silver halide emulsion layer and a color coupler which is reactive with the oxidation product of an aromatic amino developing agent to form by color development a primary dye image which absorbs a major proportion of light in one region of the visible spectrum and undesirably absorbs a minor proportion of light in at least one other region of the visible spectrum, by treating the exposed and color-developed photographic element with an oxidizing solution, such as a photographic bleaching bath, in the presence of a compound, which after oxidation couples with the residual color coupler, whereby a secondary dye image having a gradation opposite to that of said primary dye image, and absorbing light in at least one of said unwanted minor absorption regions but transmitting substantially all the light in said major absorption region is formed.

In the last mentioned pending application a method is claimed of forming a color corrected image in a photographic element having at least one silver halide emulsion

2

layer containing a color coupler which is reactive with the oxidation product of the aromatic amino developing agent to form by color development a primary dye image which absorbs a major proportion of light in one region of the visible spectrum, and undesirably absorbs a minor proportion of light in at least one other region of the visible spectrum, which method comprises treating said photographic element, after image-wise exposure and color development, with an oxidizing solution in the presence of a mask forming compound containing a grouping of the following structure:



15

wherein:

$R_1$  represents a hydrogen atom or an acyl radical such as an acetyl radical,

20  $R_2$  represents a hydrogen atom or a functional substituent which is sufficiently unstable for being split off during the oxidative coupling, such as e.g. a radical of the formula  $-\text{CONH}_2$  or  $-\text{SO}_2\text{X}$  wherein X represents a hydroxyl radical, an amino radical, a substituted amino radical such as a dialkylamino radical, an heterocyclic radical, an aliphatic hydrocarbon radical, a substituted aliphatic hydrocarbon radical, an aryl radical or a substituted aryl radical;

$R_3$  represents a hydrogen atom, an alkyl radical, an aralkyl radical, an aryl radical or a substituted aryl radical; and  $Z$  represents the non-metallic atoms necessary to complete a heterocyclic nucleus containing 5-6 members, at least one of which is a nitrogen atom.

Now we have found that color corrected images can be formed by treating an imagewise exposed photographic element comprising a silver halide emulsion layer and a color coupler which is reactive with the oxidation product of an aromatic amino developing agent to form by color development a primary dye image, after the color forming development, with an oxidizing solution, such as a photographic bleaching bath, in the presence of a compound (called hereinafter mask forming compound) corresponding to one of the following general formulae:



wherein:

55 R<sub>1</sub> represents a hydrogen atom or an acyl radical such as an acetyl radical;

56 R<sub>2</sub> represents a hydrogen atom or a functional substituent which is sufficiently unstable for being split off during the oxidative coupling, such as e.g. a radical of the formula —CONH<sub>2</sub> or —SO<sub>2</sub>X wherein X represents a hydroxyl radical, an amino radical, a substituted amino radical such as a dialkylamino radical, a heterocyclic radical such as a N-morpholinyl radical or a N-piperidyl radical, an aliphatic hydrocarbon radical, such as an alkyl radical e.g. a methyl radical or a hexadecyl radical, a substituted aliphatic hydrocarbon radical, an aryl radical, a substituted aryl radical e.g. an alkoxy substituted phenyl radical, such as a methoxy or a hexadecyloxy radical, a carboxy substituted phenyl radical, an alkyl substituted phenyl radical such as a tolyl radical, a carboxy substituted

phenyl radical, a sulphonic acid substituted phenyl radical, a sulphonic acid ester substituted phenyl radical, a sulfamoyl phenyl radical, a halogen substituted phenyl radical such as a 2,5-dichloro-phenyl radical, and an acylamino phenyl radical;

$R_3$  represents a hydrogen atom, an alkyl radical such as a methyl radical, a hexadecyl radical or an allyl radical, an aralkyl radical such as a benzyl radical, an aryl radical such as a phenyl or a naphthyl radical or a substituted aryl radical such as a methoxy substituted phenyl radical;

$R_4$  represents a hydrogen atom, an alkyl radical such as a methyl radical, a hexadecyl radical, or an allyl radical, an aralkyl radical such as a benzyl radical, an aryl radical such as a phenyl radical or a naphthyl radical or a substituted aryl radical such as a methoxy substituted phenyl radical;

$R_5$  represents a hydrogen atom, an amino radical, a substituted amino radical such as a methylphenyl amino radical, an alkyl radical such as a methyl radical or an ethyl radical, an aralkyl radical such as a

5  
10

15

20

dihalogenated phenyl radical, an hydroxy substituted phenyl radical, an alkoxy substituted phenyl radical such as a mono- or dimethoxy phenyl radical or a hexadecycloxy phenyl radical, an alkyl mercapto-phenyl radical, an acyloxyphenyl radical such as a palmitoyloxyphenyl radical, an acylaminophenyl radical, a dialkyl aminophenyl radical, such as a p-(N-methyl-N-pentadecyl)-aminophenyl radical, an alkylsulfonylphenyl radical, or a heterocyclic radical such as a furyl radical, a thienyl radical, a pyridyl radical or a 1,3-benzodioxol-5-yl radical;

$L_1$  and  $L_2$  each represents a methine group or a nitrogen atom, at least one of  $L_1$  and  $L_2$  being a methine group;  $Y$  represents the non-metallic atoms necessary to form an heterocyclic nucleus such as a morpholine nucleus or a piperidine nucleus; and

$n$  is an integer from 1 to 4.

Amidrazones which can be used as mask forming compounds in the process of the present invention and which correspond to the general Formula I are for instance the compounds listed hereinafter:

| Compound | $R_1$ | $R_2$                | $R_3$ | $R_4$           | $R_5$           | $n$     |   |
|----------|-------|----------------------|-------|-----------------|-----------------|---------|---|
| 1        | H     |                      |       | $-CH_3$         | $-C_{16}H_{33}$ |         | 1 |
| 2        | H     |                      |       | $-CH_3$         | $-C_{16}H_{33}$ |         | 1 |
| 3        | H     | $-SO_2-C_{16}H_{33}$ |       | $-CH_3$         | $-CH_2-$        |         | 1 |
| 4        | H     | $-SO_2-C_{16}H_{33}$ |       |                 |                 | 1       |   |
| 5        | H     |                      |       |                 |                 | $-CH_3$ | 1 |
| 6        | H     |                      |       | $-CH_2-CH=CH_2$ |                 |         | 1 |
| 7        | H     |                      |       | $-CH_3$         | $-C_{16}H_{33}$ |         | 1 |
| 8        | H     | $-CONH_2$            |       | $-CH_3$         | $-C_{16}H_{33}$ |         | 1 |
| 9        | H     | $-SO_2-C_{16}H_{33}$ |       | $-C_2H_5$       | $-C_2H_5$       |         | 1 |
| 10       | H     |                      |       | $-CH_3$         | $-C_{16}H_{33}$ |         | 1 |
| 11       | H     |                      |       | $-CH_3$         | $-C_{16}H_{33}$ |         | 1 |

benzyl radical, a substituted benzyl radical such as a methoxy substituted benzyl radical, an alkylene radical such as a methoxy styryl radical, an aryl radical, a substituted aryl radical such as a mono- or

75  
Amidrazones which can be used as mask forming compounds in the process of the present invention and which correspond to the general Formula II are for instance the compounds listed hereinafter:

| Compound | R <sub>1</sub> | R <sub>2</sub>                                                                                  | R <sub>3</sub>                                                                      | Y                                                                                     | n |
|----------|----------------|-------------------------------------------------------------------------------------------------|-------------------------------------------------------------------------------------|---------------------------------------------------------------------------------------|---|
| 1        | H              | -SO <sub>2</sub> -C <sub>6</sub> H <sub>4</sub> -O-C <sub>16</sub> H <sub>33</sub>              |    |    | 1 |
| 2        | H              | -SO <sub>2</sub> -C <sub>6</sub> H <sub>4</sub> -COOC <sub>2</sub> H <sub>5</sub>               |    |    | 1 |
| 3        | H              | -SO <sub>2</sub> -C <sub>6</sub> H <sub>4</sub> -COOH                                           |    |    | 1 |
| 4        | H              | -SO <sub>2</sub> -N(H <sub>2</sub> ) <sub>2</sub> C <sub>2</sub> H <sub>4</sub> CH <sub>3</sub> |   |    | 1 |
| 5        | H              | -SO <sub>2</sub> -(CH <sub>2</sub> ) <sub>10</sub> -CH <sub>3</sub>                             |    |    | 1 |
| 6        | H              | -SO <sub>2</sub> -C <sub>6</sub> H <sub>4</sub> -CH <sub>3</sub>                                |   |    | 1 |
| 7        | H              | -SO <sub>2</sub> -C <sub>6</sub> H <sub>4</sub> -C <sub>16</sub> H <sub>33</sub>                |  |  | 1 |
| 8        | H              | -SO <sub>2</sub> -CH <sub>3</sub>                                                               |  |  | 1 |
| 9        | H              | -CONH <sub>2</sub>                                                                              |  |  | 1 |
| 10       | H              | -SO <sub>2</sub> -C <sub>16</sub> H <sub>33</sub>                                               |  |  | 1 |
| 11       | H              | -SO <sub>2</sub> -C <sub>6</sub> H <sub>4</sub> -CH <sub>3</sub>                                | -CH <sub>3</sub>                                                                    |  | 1 |
| 12       | H              | -SO <sub>2</sub> -C <sub>16</sub> H <sub>33</sub>                                               |  |  | 1 |
| 13       | H              | -SO <sub>2</sub> -L(H <sub>2</sub> ) <sub>2</sub> C <sub>2</sub> H <sub>4</sub> CH <sub>3</sub> |  |  | 1 |
| 14       | H              | -SO <sub>2</sub> -C <sub>6</sub> H <sub>4</sub> -CH <sub>3</sub>                                |  |  | 1 |
| 15       | H              | -SO <sub>2</sub> -C <sub>6</sub> H <sub>4</sub> -CH <sub>3</sub>                                |  |  | 1 |
| 16       | H              | -SO <sub>2</sub> -C <sub>16</sub> H <sub>33</sub>                                               |  |  | 1 |

| Compound | R <sub>1</sub> | R <sub>2</sub>                                                                   | R <sub>3</sub> | Y | n |
|----------|----------------|----------------------------------------------------------------------------------|----------------|---|---|
| 17       | H              | -SO <sub>2</sub> -C <sub>16</sub> H <sub>33</sub>                                |                |   | 1 |
| 18       | H              | -SO <sub>2</sub> -C <sub>16</sub> H <sub>33</sub>                                |                |   | 1 |
| 19       | H              | -SO <sub>2</sub> -C <sub>6</sub> H <sub>4</sub> -CH <sub>3</sub>                 |                |   | 1 |
| 20       | H              | -SO <sub>2</sub> -C <sub>6</sub> H <sub>4</sub> -COOH                            |                |   | 1 |
| 21       | H              | -SO <sub>2</sub> -C <sub>6</sub> H <sub>4</sub> -C <sub>16</sub> H <sub>33</sub> |                |   | 1 |
| 22       | H              | -SO <sub>2</sub> -C <sub>16</sub> H <sub>33</sub>                                |                |   | 1 |
| 23       | H              | -SO <sub>2</sub> -C <sub>16</sub> H <sub>33</sub>                                |                |   | 1 |
| 24       | H              | -SO <sub>2</sub> -C <sub>16</sub> H <sub>33</sub>                                |                |   | 1 |
| 25       | H              | -SO <sub>2</sub> -C <sub>16</sub> H <sub>33</sub>                                |                |   | 1 |
| 26       | H              | -SO <sub>2</sub> -C <sub>16</sub> H <sub>33</sub>                                |                |   | 1 |
| 27       | H              | -SO <sub>2</sub> -C <sub>6</sub> H <sub>4</sub> -CH <sub>3</sub>                 |                |   | 1 |
| 28       | H              | -SO <sub>2</sub> -C <sub>6</sub> H <sub>4</sub>                                  |                |   | 1 |
| 29       | H              | -C(=O)HN <sub>2</sub>                                                            |                |   | 1 |
| 30       | H              | -SO <sub>2</sub> -C <sub>16</sub> H <sub>33</sub>                                |                |   | 1 |
| 31       | H              | -SO <sub>2</sub> -C <sub>16</sub> H <sub>33</sub>                                |                |   | 1 |
| 32       | H              | -SO <sub>2</sub> -O <sub>16</sub> H <sub>33</sub>                                |                |   | 1 |

Mask forming compounds having two groups which can be split off during the oxidative coupling are e.g.:



The amidrazone compounds having the general Formulae I and II can be synthesized according to H. Bredereck, Ber. 92, 837-849 (1959), according to the reaction scheme:



It is also possible in the second step of the above reaction scheme to replace the phenylhydrazine by hexadecylsulfonyl hydrazide whereby a non-migratory mask compound is obtained.

Although this method is useful, preference is given to the method of D. Peak, J. Chem. Soc. 1952, pp. 4067-4075, according to which thioimino esters are formed by reacting alkyl halides with thioamides; whereafter the formed thioimino ester is further transformed with semi-

carbazide or thiosemicarbazide in alkaline medium. The reaction scheme is the following:



wherein: R<sub>3</sub>, R<sub>4</sub>, and R<sub>5</sub> have the same significance as indicated in the general Formulae I and II.

On carrying out the second step of the latter reaction with hexadecylsulfonylhydrazide instead of semicarbazide a non-migratory mask compound is obtained. As starting materials thioamides can be used which are prepared according to sufficiently known methods. Examples of these methods are e.g. the method indicated as the Wilgerodt-Kindler reaction described by M. Carmack in Org. Reactions, vol. 3, p. 83/107, edited by R. Adams, John Wiley and Sons, New York (1946), and the transformation of amides into thioamides in pyridine by means of phosphorus pentasulfide described by E. Klingsberg, J.A.C.S. 73, p. 4988 (1951).

By way of example the preparations of some mask compounds of the present invention are given hereinafter.

#### PREPARATION 1

30 *N-phenyl-2,6-dimethyl-pyridone-(4)-hydrazone-dihydrochloride*

This compound can be prepared according to S. Hünig and G. Köbrich, Ann. 617, p. 194 (1958).

#### PREPARATION 2

35 *N<sup>3</sup>,N<sup>3</sup>-dimethyl-N<sup>1</sup>-n-hexadecylsulfonylformamidrazone*



40 A solution of 26 g. (0.75 mol) of n-hexadecylsulfonyl chloride in 280 cm.<sup>3</sup> of ether is added dropwise to a solution of an excess of hydrazine hydrate (40 cm.<sup>3</sup>) in 200

cm.<sup>3</sup> of ethanol at a temperature of 25° C. After stirring for 15 min., 120 cm.<sup>3</sup> of water are added to this solution. The n-hexadecylsulfonylhydrazide crystals thus obtained are sucked off and washed with a mixture of water and ethanol (1:3 by weight). After drying an recrystallization from acetonitrile, 24 g. of n-hexadecylsulfonylhydrazide melting at 89° C. are obtained.

A solution of 2.31 g. of phosphorus oxychloride (0.0050 mol) in 4 cm.<sup>3</sup> of anhydrous benzene is added 60 to a solution of 3.65 g. (0.0050 mol) of dimethylformamide in 4 cm.<sup>3</sup> of anhydrous benzene at a temperature of 20° C. This mixture is kept overnight at room temperature. Next, a suspension of 4 g. (0.0125 mol) of n-hexadecylsulfonylhydrazide in 35 cm.<sup>3</sup> of anhydrous benzene, prepared as described hereinbefore, is admixed at 20-25° C. After stirring for 5 h. and storing for 12 h., the resulting hydrochloride is precipitated with ether, sucked off and washed with ether. 5.8 g. of a hydrochloride melting at 150° C. (with decomposition) is obtained. The base is set free by introducing said hydrochloride into water, neutralizing with sodium bicarbonate and extracting with benzene. Next, this benzene solution is evaporated under reduced pressure at 40° C., and the resulting residue is washed with ethanol. 75 1.4 g. of N<sup>3</sup>,N<sup>3</sup>-dimethyl-N<sup>1</sup>-n-hexadecylsulfonyl form-

11

amidrazone melting at 89° C. are obtained. This melting point does not rise after recrystallization from methanol or free acetonitrile.

### PREPARATION 3

## *N<sup>3</sup>,N<sup>3</sup>-cyclodiethylene oxide-N<sup>1</sup>-n-hexadecylsulfonyl-thieneamidrazone*



5.6 g. (0.050 mol) of 2-thiopheno aldehyde, 2.4 g. (0.075 mol) of sulfur and 6.5 g. (0.075 mol) of morpholine are heated for 3 h. on a water-bath. After pouring the reaction mixture into 100 cm.<sup>3</sup> of water, sucking off, washing with water and drying, 11.5 g. of a product melting at 72° C. are obtained. After recrystallization from isopropanol, 7.8 g. of thiothieno morpholide melting constantly at 77° C. are obtained.

A solution of 2.13 g. (0.010 mol) of this compound in 15 cm.<sup>3</sup> of acetone is refluxed for 1 h. with 2 cm.<sup>3</sup> (0.030 mol) of methyl iodide. The resulting precipitate is sucked off and washed with acetone. 3.8 g. of 4-(alpha-methylthiothienylidene)-morpholinium iodide melting at 163° C. (with decomposition) are obtained.

1.95 g. (0.0055 mol) of this morpholinium iodide and 1.6 g. (0.005 mol) of *n*-hexadecylsulfonyl hydrazide, prepared as described in Preparation 2, are allowed to react for 24 h. at room temperature in 18 cm.<sup>3</sup> of pyridine. After pouring this reaction mixture into 100 cm.<sup>3</sup> of water, sucking off, washing with water and drying, 2 g. of a product melting at 60° C. are obtained. After recrystallization from methanol 1 g. of  $N^3,N^3$ -cyclodiethylene oxide- $N^1$ -*n*-hexadecylsulfonyl thienamidrazone melting at 78° C. is obtained.

## PREPARATION 4

*N<sup>3</sup>,N<sup>3</sup>-cyclodiethylene oxide-N<sup>1</sup>-hexadecylsulfonyl benzamidrazone*



9.65 g. (0.0275 mol) of 4-(alpha-methylthiobenzylidene)-morpholinium iodide prepared according to D. Peak, J. Chem. Soc. (1952), 4067-75, and 8 g. (0.025 mol) of n-hexadecylsulfonylhydrazide prepared according to Preparation 1, are heated for 2 h. at 50° C. in a mixture of 95 cm.<sup>3</sup> of pyridine and 5 cm.<sup>3</sup> of piperidine. Next the reaction mixture is poured out into 500 cm.<sup>3</sup> of water. The precipitate formed is sucked off, washed with water and dried. 11.7 g. of product melting unsharply at 80° C. are obtained. After recrystallization from methanol 8 g. of N<sup>3</sup>,N<sup>3</sup>-cyclodiethylene oxide-N<sup>1</sup>-n-hexadecylsulfonyl benzamidrazone melting at 94° C. for obtained.

## PREPARATION 5

*N<sup>3</sup>,N<sup>3</sup>-cyclodiethyleneoxide-N<sup>1</sup>-n-hexadecylsulfonyl phenyl acetamidrazone*



1 g. (0.0027 mol) of 4-(1-methylthio-2-phenyl ethylidene)-morpholinium iodide, prepared according to D. Peak, J. Chem. Soc. (1952), 4071, and 0.8 g. (0.0025 mol) of n-hexadecylsulfonyl hydrazide are allowed to react for 24 h. at room temperature in 20 cm.<sup>3</sup> of pyridine. After pouring this solution into water and recrystalliza-

12

tion from methanol 0.5 g. of amidrazone melting at 79° C. is obtained.

## PREPARATION 6

*N<sup>3</sup>,N<sup>3</sup>-cyclopentyl-N<sup>1</sup>-(4-carboxyphenylsulfonyl)-3-methoxy-4-n-hexadecylbenzamidrazone*



7.5 g. (0.33 mol) of sodium are dissolved in 750 cm.<sup>3</sup> of methyl Cellosolve (trade name for ethylene glycol monomethylether). After adding 50 g. (0.33 mol) of 3-methoxy-4-hydroxybenzaldehyde and refluxing the reaction mixture until complete dissolution of the reactants 90 g. (0.3 mol) of n-hexadecylbromide are dropwise added. After further heating for 1.5 h., the reaction mixture is cooled and sucked off. The filtered crystals are then recrystallized from methanol yielding 86 g. of 3-methoxy-4-n-hexadecyloxybenzaldehyde. Melting point: 69°C.

A mixture consisting of 9.4 g. (0.025 mol) of this aldehyde, 1.2 g. of flowers of sulfur and 3.7 cm.<sup>3</sup> (0.038 mol) of piperidine is heated for 6 h. on a water-bath. After cooling, the product obtained is ground under water, sucked off, washed with water and recrystallized from ethanol yielding 9.7 g. of 3-methoxy-4-n-hexadecyl-oxybenzothiopiperidine. Melting point: 67° C.

A mixture consisting of 38 g. (0.08 mol) of this compound, 16 cm.<sup>3</sup> (0.24 mol) of methyl iodide and 160 cm.<sup>3</sup> of anhydrous acetone are refluxed for 1 h. After sucking off and washing with ether 41.5 g. of 1-alpha-methylthio - 3-methoxy-4-n-hexadecyloxy benzylidene-piperidinium iodide are obtained. Melting point: 90° C. (with decomposition). On recrystallization the product is unstable.

6.17 g. (0.01 mol) of this compound dissolved in 50 cm.<sup>3</sup> of pyridine are allowed to react for 12 h. at room temperature with 2.16 g. (0.01 mol) of 4-carboxyphenyl sulfonyl hydrazide. After pouring into ice, sucking off, washing with water and recrystallization from acetonitrile, 3 g. of  $N^3,N^3$ -cyclopentyl- $N^1$ -(4-carboxyphenylsulfonyl)-3-methoxy-4-N-hexadecyloxybenzamidrazone are obtained. Melting point: 108° C.

The 4-carboxyphenyl sulfonyl hydrazide used in the above preparation is obtained by first dissolving 11 g. (0.05 mol) of 4-carboxyphenylsulfonyl chloride in 650 cm.<sup>3</sup> of anhydrous ether and by adding thereto at -5° C. 6.5 cm.<sup>3</sup> of hydrazine. After washing the precipitate with cold ethanol, the obtained salt is boiled in ethanol and then ground under 5 N hydrochloric acid for obtaining the carboxylic acid hydrazonium salt. After recrystallization of this salt from water, 6 g. of 4-carboxyphenyl sulfonyl hydrazide is obtained. Melting point: 235° C. (with decomposition).

## PREPARATION 7

***N<sup>3</sup>,N<sup>3</sup>-cyclopentyl-N<sup>1</sup>-n-hexadecylsulfonyl-3-methoxy-4-hydroxybenzamidrazone***



8.75 g. (0.0575 mol) of 3-methoxy-4-hydroxybenzaldehyde and 5 cm.<sup>3</sup> (0.050 mol) of piperidine are reacted for 8 h. at 100° C. with 2.4 g. (0.075 mol) of sulfur. The sticky mass is cooled and transformed into a powdery substance by adding water thereto. This powder is sucked off and washed with water until neutral. The crude product obtained is recrystallized from petroleum naphtha (boiling range 90°-120°) yielding 7 g. of 3-methoxy-4-hydroxybenzothiopiperide. Melting point: 118° C. Re-

crystallization from ethylacetate raises the melting point to 119° C.

15 g. (0.06 mol) of the foregoing thioamide are refluxed for 1 h. with 17 cm.<sup>3</sup> (0.28 mol) of methyl iodide in 177 cm.<sup>3</sup> of anhydrous acetone.

After cooling the reaction product is sucked off and washed with ether yielding 23 g. of 1-(alpha-methylthio-3-methoxy-4-hydroxy-benzylidene)-piperidinium iodide. Melting point: 176° C. (with decomposition). The product is unstable on recrystallization.

23 g. (0.06 mol) of the foregoing iodide salt are reacted at room temperature for 12 h. with 18.4 g. (0.06 mol) of n-hexadecyl sulfonyl hydrazide dissolved in 230 cm.<sup>3</sup> of pyridine.

After pouring out the reaction mixture on ice, the solidified product is washed with water and recrystallized from ethanol. 25 g. of N<sup>3</sup>,N<sup>3</sup>-cyclopentyl-N<sup>1</sup>-n-hexadecylsulfonyl-3-methoxy-4-hydroxybenzamidrazone are obtained. Melting point: 93° C.

#### PREPARATION 8

##### N<sup>3</sup>,N<sup>3</sup>-cyclodiethylene-oxide-N<sup>1</sup>-n-hexadecylsulfonyl-4-methoxybenzamidrazone



A mixture consisting of 13.6 g. (0.1 mol) of p-methoxybenzaldehyde, 4.8 g. (0.15 mol) of flowers of sulfur and 13 cm.<sup>3</sup> (0.15 mol) of morpholine is refluxed for 3 h. on a water-bath. After cooling, sucking off, washing with water and recrystallization from ethanol, 20.5 g. of 4-methoxybenzothiomorpholide are obtained. Melting point: 109° C. A further recrystallization does not alter the melting point.

A mixture consisting of 11.8 g. (0.05 mol) of this thiomorpholide, 50 cm.<sup>3</sup> of anhydrous acetone and 5 cm.<sup>3</sup> (0.05 mol) of methyl iodide is refluxed for 1 h. The precipitate formed is sucked off and washed with ether to yield 18.5 g. of 4-(alpha-methylthio-4-methoxybenzylidene)-morpholinium iodide. Melting point: 152° C. (with decomposition). On recrystallization this product is not stable.

1.04 g. (0.00275 mol) of this morpholinium iodide is reacted for 12 h. at room temperature in a mixture of 35 cm.<sup>3</sup> of pyridine and 0.8 g. (0.0025 mol) of n-hexadecylsulfonyl hydrazide. The reaction mixture is poured into ice. The formed crystals are sucked off, washed with water and recrystallized from ethanol to yield 1 g. of N<sup>3</sup>,N<sup>3</sup>-cyclodiethylene oxide-N<sup>1</sup>-n-hexadecylsulfonyl-4-methoxybenzamidrazone. Melting point: 69° C.

#### PREPARATION 9

##### N<sup>3</sup>,N<sup>3</sup>-cyclodiethylene oxide-N<sup>1</sup>-n-hexadecylsulfonyl-2,4-dichlorobenzamidrazone



To a chilled solution of 6 g. (0.15 mol) of sodium hydroxide in 50 cm.<sup>3</sup> of water are first added at 0° C. 11 g. (0.125 mol) of morpholine, and then at 0° to 5° C. 26.2 g. (0.125 mol) of 2,4-dichlorobenzoylchloride. After adding the reactants the reaction mixture is stirred for another hour at the same temperature. After sucking off, washing until neutral with water and recrystallization from petroleum naphtha, 24 g. of 2,4-dichlorobenzomorpholide are obtained. Melting point: 94° C.

5.2 g. (0.02 mol) of this morpholide in a mixture of 25 cm.<sup>3</sup> of pyridine and 1.8 g. (0.008 mol) of phosphorus pentasulfide are refluxed for 40 min. After pouring the reaction mixture into ice the formed precipitate is sucked

off, washed with water and recrystallized from ethanol to yield 4.5 g. of 2,4-dichlorobenzothiomorpholide. Melting point: 148° C.

34.5 g. (0.125 mol) of this thiomorpholide dissolved in 22.5 cm.<sup>3</sup> (0.375 mol) of methyl iodide are refluxed for 1 h. After sucking off, 20 g. of 4-(alpha-methylthio-2,4-dichlorobenzylidene)-morpholinium iodide are obtained. Melting point: 160° C. (with decomposition). This product is unstable on recrystallization.

55 g. (0.13 mol) of this product dissolved in 750 cm.<sup>3</sup> of pyridine are reacted at room temperature for 48 h. with 39 g. (0.12 mol) of n-hexadecylsulfonylhydrazide. After pouring this reaction mixture into ice, sucking off, washing with water and recrystallization, 54 g. of N<sup>3</sup>,N<sup>3</sup>-cyclodiethylene oxide-N<sup>1</sup>-n-hexadecylsulfonyl-2,4-dichlorobenzamidrazone are obtained. Melting point: 70° C.

#### PREPARATION 10

##### N<sup>3</sup>-methyl-N<sup>3</sup>-phenyl-N<sup>1</sup>-n-hexadecylsulfonylbenzamidrazone



8 g. (0.022 mol) of N-methyl-alpha-methylthiobenzylidene anilinium iodide prepared according to D. Peak, J.C.S. (1952), p. 4071, are reacted for 24 h. with 6.4 g.

30 (0.02 mol) of n-hexadecylsulfonylhydrazide in 60 cm.<sup>3</sup> of pyridine. The reaction mixture is poured on ice, the precipitate formed is sucked off, washed with water and finally washed with methanol. After recrystallizing from methanol 7 g. N<sup>3</sup>-methyl-N<sup>3</sup>-phenyl-N<sup>1</sup>-n-hexadecylsulfonylbenzamidrazone are obtained. Melting point: 72° C.

#### PREPARATION 11

##### N<sup>3</sup>,N<sup>3</sup>-cyclodiethyleneoxide-N<sup>1</sup>-n-hexadecylsulfonyl-2-chlorobenzamidrazone



45 To a chilled solution of 6 g. (0.15 mol) of sodium hydroxide in 50 cm.<sup>3</sup> of water are first added at 0° C. 11 g. (0.125 mol) of morpholine and then at 0° to 5° C. 22 g. (0.125 mol) of o-chlorobenzoylchloride. After the addition of the reactants stirring is continued for 1/2 h. at the same temperature. The product formed is filtered off and washed with water until neutral. Recrystallization from petroleum naphtha yields 20 g. of 2-chlorobenzomorpholide. Melting point: 73° C.

55 14.5 g. (0.065 mol) of the preceding amide are reacted at reflux temperature for 40 min. with 5.8 g. (0.026 mol) of phosphorus pentasulfide in 65 cm.<sup>3</sup> of pyridine. After pouring out the reaction mixture in ice, sucking off, washing with water and recrystallizing from ethanol 11 g.

60 of 2-chlorobenzothiomorpholide are obtained. Melting point: 124° C.

65 11 g. (0.045 mol) of the preceding thioamide are refluxed for 1 h. with 8.8 cm.<sup>3</sup> (0.15 mol) of methyl iodide in 40 cm.<sup>3</sup> of anhydrous acetone. After cooling, the formed reaction product is sucked off and washed with ether to yield 16 g. of 4-(alpha-methylthio-2-chlorobenzylidene)-morpholinium iodide. Melting point: 152° C. (with decomposition). The product cannot be recrystallized because it is not stable enough.

70 16 g. (0.04 mol) of the preceding morpholinium iodide are reacted at room temperature for 48 h. with 11.5 g. (0.036 mol) of n-hexadecylsulfonylhydrazide in 220 cm.<sup>3</sup> of pyridine. The reaction mixture is poured into ice and the precipitate formed is sucked off, washed with water and recrystallized from n-hexane to yield 17 g. of N<sup>3</sup>,N<sup>3</sup>-

15

cyclodiethyleneoxide- $N^1$  - n - hexadecylsulfonyl-2-chlorobenzamidrazone. Melting point: 75° C.

## PREPARATION 12

$N^3$ -methyl- $N^3$ -n-hexadecyl- $N^1$ -(4'-carboxyphenylsulfonyl)-3,4-dimethoxybenzamidrazone



To a solution of 25.5 g. (0.1 mol) of methyl-n-hexadecylamine in a mixture of 250 cm.<sup>3</sup> of dioxane and 22.5 cm.<sup>3</sup> (0.11 mol) of 5 N sodium hydroxide is added dropwise at 20° C. a solution of 20.5 g. (0.1 mol) of 3,4-dimethoxybenzoylchloride in 50 cm.<sup>3</sup> of dioxane. After stirring this mixture for 1 h. 125 cm.<sup>3</sup> of water are added. The formed oily layer is dried on sodium sulfate and distilled under reduced pressure. Boiling point: 236-240° C., 0.4 mm. of Hg pressure. Yield: 34 g. of 3,4-dimethoxybenzoic acid-methyl-n-hexadecylamide.

45 g. (0.1 mol) of the preceding amide are refluxed for 2 h. with 24 g. (0.1 mol) of phosphorus pentasulfide in 100 cm.<sup>3</sup> of pyridine. After pouring into ice and adding sodium chloride, the coagulated product is sucked off, washed with water and recrystallized from acetonitrile to yield 34 g. of 3,4-dimethoxybenzothio-methyl-n-hexadecylamide. Melting point: 63° C.

10 g. (0.023 mol) of the preceding thioamide are dissolved at room temperature in 10 cm.<sup>3</sup> of methyl iodide. Immediately after complete dissolution ether is added and the solution is left for 12 h. in a refrigerator. 6.1 g. of alpha-methylthio-3,4-dimethoxybenzylidene-methyl-n-hexadecylammonium iodide are obtained. Melting point: 100° C. (with decomposition). The product is unstable and cannot be purified by recrystallization.

13.5 g. (0.0234 mol) of the preceding compound are allowed to react for 72 h. at room temperature in 50 cm.<sup>3</sup> of pyridine with 5.05 g. (0.0234 mol) of 4-carboxyphenylsulfonylhydrazide. The solvent is distilled off and the residue is left under water to solidify. The solidified product is freed from water by sucking off and recrystallized from ethanol to yield 8 g. of  $N^3$ -methyl- $N^3$ -n-hexadecyl- $N^1$ -(4'-carboxyphenylsulfonyl)-3,4-dimethoxybenzamidrazone. Melting point: 142° C.

## PREPARATION 13

$N^3$ -methyl- $N^3$ -n-hexadecyl- $N^1$ -(4'-tolusulfonyl)-4-methoxybenzamidrazone



61 g. (0.24 mol) of methyl-n-hexadecylamine are dissolved at 30° C. in a mixture of 18 g. (0.48 mol) of sodium hydroxide, 180 cm.<sup>3</sup> of water and 1200 cm.<sup>3</sup> of dioxane. Whilst stirring at 10° C., 41 g. (0.24 mol) of p-methoxybenzoylchloride are added dropwise to the reaction mixture and stirring is continued thereafter for 1 h. The reaction mixture is poured on ice, and the solid product formed is sucked off and washed with water. Recrystallization from a mixture ethanol/water (6:1) yields 70 g. of p-methoxybenzoyl-N-methyl-N-n-hexadecylamide. Melting point: 50° C.

15 g. (0.04 mol) of this amide are refluxed for 40 min. with 4 g. (0.016 mol) of phosphorus pentasulfide in 150 cm.<sup>3</sup> of pyridine. The reaction mixture is poured on ice and the solidified material formed is sucked off, washed with water and recrystallized from ethanol to yield 13.5

70

g. of 4-methoxybenzothio-N-methyl-N-n-hexadecylamide. Melting point: 63° C.

13.5 g. (0.033 mol) of this thioamide are refluxed for 1 h. with 13.5 cm.<sup>3</sup> (0.022 mol) of methyl iodide in 70 cm.<sup>3</sup> of acetone. After distilling off the solvent and washing the residue with the ether, 17 g. of alpha-methylthio-4-methoxybenzylidene-methyl-n-hexadecyl ammonium iodide are obtained. Melting point: 75° C. (with decomposition). This product is not stable enough for being purified by recrystallization.

11 g. (0.02 mol) of this compound are reacted for 12 h. at room temperature with 3.7 g. (0.02 mol) of p-tolusulfonylhydrazide in 70 cm.<sup>3</sup> of pyridine. The reaction mixture is poured on ice. The precipitate formed is washed with water and recrystallized from methanol to yield 8 g. of  $N^3$ -methyl- $N^3$ -n-hexadecyl- $N^1$ -(4'-tolusulfonyl)-4-methoxybenzamidrazone. Melting point: 66° C.

15

## PREPARATION 14

$N^3$ -phenyl- $N^3$ -allyl- $N^1$ -(4'-tolusulfonyl)-benzamidrazone



To a boiling solution of 13.3 g. (0.1 mol) of  $N$ -allylaniline in toluene is dropwise added a solution of 14 g. (0.1 mol) of benzoylchloride in 50 cm.<sup>3</sup> of toluene in such a rate that the toluene on being distilled over carries off the formed hydrogen chloride. This reaction is continued for 8 h., during which period toluene is added for maintaining the liquid volume constant. After distilling off the solvent the residue is distilled under reduced pressure to yield 15 g. of  $N$ -allylbenzalanilide. Boiling range: 134-138° C./0.6 mm. of Hg pressure.

76 g. (0.32 mol) of this anilide are allowed to react for 40 min. with 44.5 g. (0.2 mol) of phosphorus pentasulfide in 450 cm.<sup>3</sup> of pyridine. The reaction mixture is poured on ice, washed with a sodium sulfide solution and with water. Recrystallization from n-hexane yields 57 g. of  $N$ -allylbenzothioanilide. Melting point: 69° C.

5 g. (0.02 mol) of this thioanilide are reacted for 12 h. at room temperature with 15 cm.<sup>3</sup> of methyl iodide. After sucking off the solid product and washing with acetone, 7.2 g. of alpha-methylthiobenzylidene- $N$ -allylanilinium iodide are obtained. Melting point: 180° C. (with decomposition). For the product is not stable enough it cannot be purified by recrystallization.

4 g. (0.01 mol) of the preceding compound and 1.7 g. (0.03 mol) of potassium hydroxide dissolved in 40 cm.<sup>3</sup> of anhydrous ethanol are reacted for 24 h. at room temperature with 1.86 g. (0.01 mol) of p-tolusulfonylhydrazide. After evaporating under reduced pressure at 30° C., the residue is first washed with water and next with ethanol in order to obtain a solid product. After recrystallization from methanol 1.3 g. of  $N^3$ -phenyl- $N^3$ -allyl- $N^1$ -(4'-tolusulfonyl)-benzamidrazone are obtained. Melting point: 140° C.

70

## PREPARATION 15

$N^3$ ,  $N^3$ ,  $N^3$ ,  $N^3$ -diethylene-di( $N^1$ -n-hexadecylsulfonylbenzamidrazone)



88.2 g. (0.3 mol) of dibenzoylpiperazine prepared according to A. V. Hofmann, Ber. 23, 3301 (1890), are re-

fluxed for 2 h. with 80 g. (0.36 mol) of phosphorus pentasulphide in 200 cm.<sup>3</sup> of pyridine. The reaction mixture is poured on ice, sucked off, washed with an aqueous sodium sulphide solution and with water. By boiling the washed precipitate in carbon disulphide and by recrystallizing from dichloroethane 65 g. of dibenzothiopiperazide are obtained. Melting point: 275° C. (unsharp).

1.83 g. (0.005 mol) of this product is refluxed for 1 h. with 3.6 cm.<sup>3</sup> (0.06 mol) of methyl iodide in 40 cm.<sup>3</sup> of dichloroethane. The reaction mixture is sucked off and the solid product obtained is washed with dichloroethane to yield 3.1 g. of 1,4-di(2-methylthio-benzylidene)-piperazonium iodide. Melting point: 190° C. (with decomposition). This product is unstable and cannot be purified by recrystallization.

7.2 g. (0.12 mol) of the foregoing compound are allowed to react for 24 h. at room temperature with 7.5 g. (0.24 mol) of n-hexadecylsulfonyl-hydrazide in 150 cm.<sup>3</sup> of pyridine. The reaction mixture is poured on ice, the solid product formed is sucked off, washed with water and next with methanol. Recrystallization from methyl-ethyl-ketone yields 7 g. of N<sup>3</sup>, N<sup>3</sup>, N'<sup>3</sup>, N'<sup>3</sup> - diethylene - di (N<sup>1</sup> - n - hexadecylsulfonylbenzamidrazone). Melting point: 141° C.

#### PREPARATION 16

##### N,N'-dimethyl-N,N'-diphenyl-N''-aminoguanidine



A solution in 15 cm.<sup>3</sup> of warm ethanol of 1.99 g. (0.005 mol) of N,N'-dimethyl-N,N'-diphenyl-S-methyl-isothiouronium iodide, prepared according to D. Peak, J. Chem. Soc., 4072 (1952), is dropwise added to 0.25 cm.<sup>3</sup> (0.005 mol) of hydrazine hydrate whilst heating on a water-bath. Heating is continued for 2 h. and air is bubbled through the reaction mixture until no more methylmercaptane is formed. After evaporation to dryness, the residue is washed with ether and recrystallized from isopropanol. 1 g. of N,N'-dimethyl-N,N'-diphenyl-N''-amino-guanidine is obtained. Melting point: 182° C.

According to a preferred embodiment of the present invention, the mask forming compound is incorporated in one of the layers present in the light sensitive photographic material, preferably in the silver halide emulsion layer wherein the mask image is to be formed by oxidative coupling of the residual color coupler, present in that layer, with the mask forming substance; in order to prevent the diffusion of the mask forming compound out of the silver halide emulsion layer wherein this compound originally was incorporated, preferably mask forming compounds are used containing a radical (e.g. the radical X and/or R<sub>3</sub> in the above formulae) comprising a linear chain of 5 to 20 carbon atoms.

The process of color correction of the present invention may be practised i.e. by using a color photographic material containing a coupler for magenta belonging to the class of the pyrazolone or indazolone color couplers and/or a coupler for cyan belonging to the class of the phenol or naphthol color couplers. Depending upon the structure of the color coupler used in combination with the mask-forming compound according to the present invention, yellow to magenta colored mask images are obtained on treating the photographic material with an oxidizing substance such as present in a potassium ferricyanide bleaching bath.

It has been found that by oxidative coupling of the mask-forming compounds of the Formula II above with a pyrazolone or indazolone color coupler for magenta, a yellow colored mask image is obtained which compensates the undesirable side-absorption in the blue part of the spectrum of the magenta dye image obtained by

color development of the exposed areas of the layer containing said coupler for magenta.

It has further been found that by oxidative coupling of the mask-forming compounds of the Formula I or II above with naphthol color couplers for cyan, a yellow to magenta colored mask image is obtained which compensates the undesirable side-absorption in the blue and green part of the spectrum of the cyan image obtained by color development of the exposed areas of the layer containing said cyan coupler. Naphthol color couplers which are especially useful for obtaining a mask image by reaction with the mask forming substances according to the present invention are e.g. those represented by the general formula:

15

20



wherein:

- 25 X represents a member selected from the group consisting of an oxygen atom, a sulfur atom, a —NH—CO— group, a —CO—NH group, a —SO<sub>2</sub>—NH— group, a —NH—SO<sub>2</sub>— group, a —N-alkyl group and a sulfonyl group;
- 30 Z represents a member selected from the group consisting of a hydrogen atom and a halogen atom;
- D represents an aliphatic radical comprising a linear chain of at least 5 and at most 20 carbon atoms, preferably 14, 16 or 18 carbon atoms;
- 35 M represents a member selected from the group consisting of a hydrogen atom, an alkali metal atom and an ammonium group.

Suitable color couplers of the above general formula are for instance:

- 40 N-(2'-n-hexadecyloxy-5'-sulfo) - phenyl - 1 - hydroxy-2-naphthoic acid amide sodium salt,  
N-(2'-n-hexadecyloxy - 5' - sulfo) - phenyl-1-hydroxy-4-chloro-2-naphthoic acid amide sodium salt,  
45 N-(2'-n-hexadecylmercapto-5'-sulfo) - phenyl-1-hydroxy-2-naphthoic acid amide sodium salt,  
N-(2'-n-hexadecylmercapto-5'-sulfo) - phenyl-1-hydroxy-4-bromo-2-naphthoic acid amide sodium salt,  
50 N-(2'-n-hexadecylmercapto-5'-sulfo) - phenyl-1-hydroxy-4-chloro-2-naphthoic acid amide sodium salt,  
N-(2'-palmitylamino - 4' - sulfo) - phenyl-1-hydroxy-2-naphthoic acid amide sodium salt,  
55 N-(2'-methyl cetylamino-5'-sulfo)-phenyl - 1 - hydroxy-4-chloro-2-naphthoic acid amide sodium salt,  
N-(6'-n-hexadecylsulfonylphenyl)-1-hydroxy - 2 - naphthoic acid amide-3'-sodium sulfonate,  
N-(6'-n-hexadecylsulfonylphenyl) - 1 - hydroxy-4-chloro-2-naphthoic acid amide-3'-sodium sulfonate,  
60 N-(4'-n - hexadecylsulfonyl)-1-hydroxy-2-naphthoic acid amide-3'-sodium sulfonate.

These color couplers for cyan can be prepared e.g. by condensation of 1-hydroxy-2-naphthoic acid or its derivatives with the suitable aromatic amines according to 65 U.S. patent application Serial No. 66,289, filed October 31, 1960, by Arthur Henri de Cat, Raphael Karel Van Poucke and Hector Alfons Van den Eynde.

It is to be noted that by oxidative coupling of some 70 of the amidrazone mask forming compounds of the Formula I or II above with color couplers for cyan of the formula given above, a yellow to orange colored mask image is obtained which compensates the undesirable side-absorption in the blue as well as in the green part of the spectrum.

For carrying out the process according to the present invention, the color couplers and mask compounds can be incorporated into a photographic silver halide emulsion prepared by means of the colloids usually employed therefor, such as for instance gelatin, polyvinyl alcohol, collodion or other natural or synthetic colloids. The silver halide emulsion can be coated on a support consisting of paper, glass, nitrocellulose, cellulose esters such as cellulose triacetate, polyester, polystyrene or another natural or synthetic resin, and forms part of a photographic material with one or more emulsion layers. The multilayer material usually comprises the following elements: a support, a red-sensitive emulsion layer having a color coupler for cyan, a green-sensitive emulsion layer having a color coupler for magenta and a blue-sensitive emulsion layer having a color coupler for yellow. There is a yellow filter composed in most of the cases of a gelatin layer containing dispersed colloidal silver, located between the blue-sensitive emulsion layer and the green-sensitive emulsion layer. It is not only possible to incorporate the color couplers into the light-sensitive silver halide emulsion layer itself but they can also be incorporated into an adjacent non-light-sensitive colloid layer or into a non-light-sensitive layer which is separated from the light-sensitive emulsion layer by a water-permeable colloid layer.

The process according to the invention proceeds as follows: silver halide is reduced to silver at the exposed areas in a color developing bath containing a primary amine aromatic developing agent which is at the same time oxidized. The oxidized developing agent reacts with the color coupler and forms a dyestuff, the mask forming compound according to the invention not being affected. After the color development, the material comes into the bleaching bath wherein the oxidation of the mask forming compound takes place. The remaining color coupler still available at the non-exposed areas of the material couples oxidatively with the oxidation product of the compound thus formed whereby the colored mask is formed. Subsequently, the photographic color material is washed with water, fixed and dried.

The following aromatic amino-compounds can be used as developers for such material: mono-, di- and tri-amino-aryl compounds, more especially N,N-dialkyl-p-phenylenediamines, such as N,N-diethyl-p-phenylenediamine and N,N-diethyl-2-methyl-p-phenylene diamine, and derivatives thereof such as N,N-dialkyl-N'-sulfo-methyl- or carboxymethyl-p-phenylenediamine. As useful monoamino-developers should be cited: aminophenols and aminocresols or their halogen derivatives and also the amino-naphthols.

The bleaching bath generally contains potassium bromide, borax, magnesium sulfate and especially potassium ferricyanide. These elements are dissolved in precisely determined amounts of water so that a solution with a determined pH value is obtained.

The following examples illustrate the invention without limiting, however, the scope thereof.

#### EXAMPLE I

To  $\frac{1}{2}$  kg. of a red-sensitive silver bromo-iodide (2% iodide) emulsion containing  $\frac{1}{6}$  mol of silver halide are added: (1) a 10% aqueous solution containing as a color coupler for cyan 7 g. of 1,2-hydroxy-naphthoic acid-4'-sulfo-2'-n-hexadecylsulfonyl anilide, prepared according to a method described in our Belgian patent specification No. 584,846, and 5 cm.<sup>3</sup> of 2 N sodium hydroxide, and (2) 2 g. of  $N^3,N^3$ -cyclodiethylene oxide- $N^1$ -hexadecylsulfonyl benzamidrazone prepared as described in Preparation 4, dissolved in 10 cm.<sup>3</sup> of ethylene glycol monomethylether. Next, the emulsion is acidified with N acetic acid to pH=5.8 and brought to a volume of 1 litre by admixing water. After coating this emulsion onto a film support, the light-sensitive material thus obtained is exposed through a grey-wedge with a constant 0.15, and

then developed for 9 minutes at 20° C. in a color developing bath of the following composition:

|                                                | G.  |
|------------------------------------------------|-----|
| Sodium hexametaphosphate                       | 2   |
| 5 N,N-diethyl-p-phenylenediamine hydrochloride | 3   |
| Sodium sulfite                                 | 4   |
| Sodium carbonate                               | 57  |
| Hydroxylamine hydrochloride                    | 1.5 |
| Potassium bromide                              | 1   |
| 10 Water to 1000 cm. <sup>3</sup> (pH: 10.6).  |     |

This material is rinsed for 30 minutes at 18 to 20° C. and fixed for 5 minutes at 20° C. in a fixing bath of the following composition:

|                                            | G.  |
|--------------------------------------------|-----|
| 15 Sodium thiosulfate                      | 200 |
| Sodium bisulfite                           | 25  |
| Potassium alum                             | 20  |
| Sodium biacetate                           | 20  |
| Boric acid                                 | 7.5 |
| 20 Water to 1000 cm. <sup>3</sup> (pH: 4). |     |

Next, the material is rinsed again for 10 minutes at 18 to 20° C. and treated for 5 minutes in a bleaching bath of the following composition:

|                                              | G.  |
|----------------------------------------------|-----|
| Potassium ferricyanide                       | 100 |
| Potassium bromide                            | 15  |
| Borax                                        | 20  |
| Magnesium sulfate                            | 50  |
| 30 Water to 1000 cm. <sup>3</sup> (pH: 8.6). |     |

Rinsing is continued for another 10 minutes at 18 to 20° C. and then the material is fixed again for 5 minutes at 20° C. in a bath of the following composition:

|                                              | G.  |
|----------------------------------------------|-----|
| 35 Sodium thiosulfate                        | 130 |
| Borax                                        | 20  |
| Magnesium sulfate                            | 50  |
| 40 Water to 1000 cm. <sup>3</sup> (pH: 8.9). |     |

Finally, rinsing is continued for 10 minutes at 18 to 20° C. and the material is dried. The strip of finished light-sensitive color material shows in addition to a cyan wedge a red masking wedge of opposite gradation, by which the side-absorptions of the cyan image are compensated.

#### EXAMPLE 2

To  $\frac{1}{2}$  kg. of a green-sensitive silver bromo-iodide (2% iodide) emulsion containing  $\frac{1}{6}$  mol of silver halide is added an alcoholic solution of 6 g. of 1-(4'-sulfophenyl)-3-pentadecyl-pyrazolone-(5), prepared analogously to the method of Example 2 of British specification 502,665, and 2 g. of  $N^3,N^3$ -cyclodiethylene oxide- $N^1$ -hexadecylsulfonyl benzamidrazone prepared according to Preparation 4. After adding the usual additives the emulsion is coated, exposed, developed and further treated as indicated in Example 1. The finished strip shows in addition to a magenta wedge a yellow masking wedge of opposite gradation reducing the disturbing influence of the side adsorption in the formed magenta image.

#### EXAMPLE 3

To  $\frac{1}{2}$  kg. of a red-sensitive bromo-iodide emulsion (3% iodide) containing  $\frac{1}{6}$  mol of silver halide are added: (1) 9 g. of N-(6'-cetylulfonylphenyl)-1-hydroxy-2-naphthoic acid amide-3'-sodium sulfonate dissolved in a mixture of 193 cm.<sup>3</sup> of water and 7 cm.<sup>3</sup> of aqueous 2 N sodium hydroxide, and (2) 6 g. of the mask compound prepared according to Preparation 11, dissolved in a mixture of 6 cm.<sup>3</sup> of 2 N sodium hydroxide, 6 cm.<sup>3</sup> of ethanol and 18 cm.<sup>3</sup> of distilled water. After acidification to pH 6, the usual additives such as hardeners, wetting agents and stabilizers and the necessary quantity of distilled water are added to the emulsion in order to obtain 1 kg. of flowable emulsion. The emulsion is coated on a suit-

able support and dried. After exposure through a grey-wedge with a constant 0.15, the photographic material composed in this way is developed and further treated as in Example 1. In the exposed and processed strip, in addition to a cyan image also an orange to yellow mask image is formed, with a gradation opposed to that of the cyan image, and which compensates the side-absorptions of the cyan image in the blue as well as in the green region of the spectrum.

## EXAMPLE 4

To  $\frac{1}{2}$  kg. of a red-sensitive bromo-iodide emulsion (3% iodide) containing  $\frac{1}{6}$  mol of silver halide are added: (1) 9 g. of N-(6'-n-hexadecylsulfonylphenyl)-1-hydroxy-2-naphthoic acid amide-3'-sodium sulfonate dissolved in a mixture of 193 cm.<sup>3</sup> of water and 7 cm.<sup>3</sup> of aqueous 2 N sodium hydroxide, and (2) 6 g. of the mask compound prepared according to Preparation 4, dissolved in a mixture of 12 cm.<sup>3</sup> of 2 N sodium hydroxide and 18 cm.<sup>3</sup> of ethanol. After acidification to pH 6, the usual additives such as hardeners, wetting agents and stabilizers, and the necessary quantity of distilled water are added to the emulsion in order to obtain 1 kg. of flowable emulsion. The emulsion is coated on a suitable support and dried. After exposure through a grey-wedge with a constant 0.15, the photographic material composed in this way is developed and further treated as in Example 1. In the exposed and processed strip, in addition to a cyan image also an orange to yellow mask image is formed, with a gradation opposed to that of the cyan image, and which compensates the side-absorptions of the cyan image chiefly in the blue region of the spectrum.

## EXAMPLE 5

To  $\frac{1}{2}$  kg. of a red-sensitive bromo-iodide emulsion (3% iodide) containing  $\frac{1}{6}$  mol of silver halide are added: (1) 9 g. of N-(6'-n-hexadecylsulfonylphenyl)-1-hydroxy-2-naphthoic acid amide-3'-sodium sulfonate dissolved in a mixture of 193 cm.<sup>3</sup> of water and 7 cm.<sup>3</sup> of aqueous 2 N sodium hydroxide, and (2) 6 g. of the mask compound prepared according to Preparation 9, dissolved in a mixture of 6 cm.<sup>3</sup> of 2 N sodium hydroxide, 6 cm.<sup>3</sup> of ethanol and 18 cm.<sup>3</sup> of distilled water. After acidification to pH 6, the usual additives such as hardeners, wetting agents and stabilizers and the necessary quantity of distilled water are added to the emulsion in order to obtain 1 kg. of flowable emulsion. The emulsion is coated on a suitable support and dried. After exposure through a grey-wedge with a constant 0.15, the photographic material composed in this way is developed and further treated as in Example 1. In the exposed and processed strip, in addition to a cyan image also an orange to yellow mask image is formed, with a gradation opposed to that of the cyan image, and which compensates the side-absorption of the cyan image in the blue as well as in the green region of the spectrum.

## EXAMPLE 6

To  $\frac{1}{2}$  kg. of a red-sensitive bromo-iodide emulsion (3% iodide) containing  $\frac{1}{6}$  mol of silver halide are added: (1) 9 g. of N-(6'-n-hexadecylsulfonylphenyl)-1-hydroxy-2-naphthoic acid amide-3'-sodium sulfonates dissolved in a mixture of 193 cm.<sup>3</sup> of water and 7 cm.<sup>3</sup> of aqueous 2 N sodium hydroxide, and (2) 2 g. of the mask compound prepared according to Preparation 7, dissolved in a mixture of 17.5 cm.<sup>3</sup> of diacetone alcohol and 2.5 cm.<sup>3</sup> of alcoholic N/2 sodium hydroxide. After acidification to pH 6, the usual additives such as hardeners, wetting agents and stabilizers and the necessary quantity of distilled water are added to the emulsion in order to obtain 1 kg. of flowable emulsion. The emulsion is coated on a suitable support and dried. After exposure through a grey-wedge with a constant 0.15, the photographic material composed in this way is developed and further treated as in Example 1. In the exposed and processed strip, in addition to a cyan image also an orange one is formed, with a gradation

opposed to that of the cyan image, and which compensates the side-absorptions of the cyan image in the blue as well as in the green region of the spectrum.

## EXAMPLE 7

5 To  $\frac{1}{2}$  kg. of a red-sensitive bromo-iodide emulsion (3% iodide) containing  $\frac{1}{6}$  mol of silver halide are added: (1) 9 g. of N-(6'-n-hexadecylsulfonylphenyl)-1-hydroxy-2-naphthoic acid amide-3'-sodium sulfonate dissolved in a mixture of 193 cm.<sup>3</sup> of water and 7 cm.<sup>3</sup> of aqueous 2 N sodium hydroxide, and (2) 6 g. of the mask compound prepared according to Preparation 8, dissolved in a mixture of 6 cm.<sup>3</sup> of 2 N sodium hydroxide and 24 cm.<sup>3</sup> of ethanol. After acidification to pH 6 the usual additives such as hardeners, wetting agents and stabilizers and the necessary quantity of distilled water are added to the emulsion in order to obtain 1 kg. of flowable emulsion. The emulsion is coated on a suitable support and dried. After exposure through a grey-wedge with a constant 0.15, the photographic material composed in this way is developed and further treated as in Example 1. In the exposed and processed strip, in addition to a cyan image also an orange to magenta mask image is formed, with a gradation opposed to that of the cyan image, and which compensates the side-absorptions of the cyan image in the blue and the green region of the spectrum.

## EXAMPLE 8

To  $\frac{1}{2}$  kg. of a red-sensitive bromo-iodide emulsion (3% iodide) containing  $\frac{1}{6}$  mol of silver halide are added: (1) 9 g. of N-(6'-n-hexadecylsulfonylphenyl)-1-hydroxy-2-naphthoic acid amide-3'-sodium sulfonate dissolved in a mixture of 193 cm.<sup>3</sup> of water and 7 cm.<sup>3</sup> of aqueous 2 N sodium hydroxide, and (2) 3 g. of the mask compound prepared according to Preparation 6, dissolved in a mixture of 3 cm.<sup>3</sup> of 2 N sodium hydroxide, 3 cm.<sup>3</sup> of ethanol, and 9 cm.<sup>3</sup> of distilled water. After acidification to pH 6, the usual additives such as hardeners, wetting agents and stabilizers, and the necessary quantity of distilled water are added to the emulsion in order to obtain 1 kg. of flowable emulsion. The emulsion is coated on a suitable support and dried. After exposure through a grey-wedge with a constant 0.15, the photographic material composed in this way is developed and further treated as in Example 1. In the exposed and processed strip, in addition to a cyan image also an orange to magenta mask image is formed, with a gradation opposed to that of the cyan image, and which compensates the side-absorptions of the cyan image in the blue and the green regions of the spectrum.

## EXAMPLE 9

To a  $\frac{1}{2}$  kg. of red-sensitive silver bromo-iodide emulsion (2% iodide) containing  $\frac{1}{6}$  mol of silver halide are added: (1) 10 g. of N-(6'-n-hexadecylsulfonylphenyl)-1-hydroxy-2-naphthoic acid amide-3'-sodium sulfonate dissolved in a mixture of 193 cm.<sup>3</sup> of water and 7 cm.<sup>3</sup> of aqueous 2 N sodium hydroxide, and (2) 6 g. of the mask compound prepared according to Preparation 11, dissolved in a mixture of 6 cm.<sup>3</sup> of 2 N sodium hydroxide, 6 cm.<sup>3</sup> of ethanol and 18 cm.<sup>3</sup> of distilled water. After acidification to pH 6, the usual additives such as hardeners, wetting agents and stabilizers, and the necessary quantity of distilled water are added to the emulsion in order to obtain 1 kg. of flowable emulsion. After coating this emulsion forms part of a multilayer photographic material consisting of the following superposed layers in the indicated sequence: a support, an anti-halation layer, a gelatin insulating layer, the above-mentioned red-sensitive emulsion layer containing a color coupler for cyan, a gelatin interlayer, a green sensitive emulsion layer containing a color coupler for magenta, a yellow filter layer, a blue-sensitive emulsion layer containing a color coupler for yellow and at last a gelatin overcoat as antistres layer. After exposure through a grey-wedge the photographic material is developed and further treated as in Example 1. A

mainly cyan-colored image is obtained together with an orange to yellow dye image in the red-sensitive layer, said orange to yellow dye image being of opposite gradation in respect of the cyan dye image and compensating the side-absorption of the cyan image in the blue as well as in the green region of the spectrum.

## EXAMPLE 10

A photographic multilayer material consisting of the following superposed layers in the indicated sequence: a support, an anti-halation layer, a gelatin insulating layer, a red-sensitive emulsion layer containing a color coupler for cyan, a gelatin interlayer, a green-sensitive emulsion layer containing a color coupler for magenta, a yellow filter layer, a blue-sensitive emulsion layer containing a color coupler for yellow and at last a gelatin overcoat as antistress layer. The red-sensitive emulsion layer is coated starting from a red-sensitized gelatino silver bromo-iodide emulsion. This emulsion is prepared as follows: to  $\frac{1}{2}$  kg. of a gelatino silver bromo-iodide emulsion (2% iodide) containing  $\frac{1}{6}$  mol of silver halide are added: (1) 9 g. of N-(6'-n-hexadecylsulfonylphenyl)-1-hydroxy-2-naphthoic acid amide-3'-sodium sulfonate dissolved in a mixture of 175 cm.<sup>3</sup> of water and 6.3 cm.<sup>3</sup> of aqueous 2 N sodium hydroxide, and (2) 6 g. of the mask compound prepared according to Preparation 11, dissolved in a mixture of 6 cm.<sup>3</sup> of 2 N sodium hydroxide, 6 cm.<sup>3</sup> of ethanol and 18 cm.<sup>3</sup> of distilled water. Next, this emulsion is acidified with acetic acid to pH 6, and after adding the usual additives such as hardeners, wetting agents, stabilizers and the necessary quantity of distilled water, 1 kg. of flowable emulsion is obtained. The green-sensitive emulsion layer is coated starting from a green-sensitized gelatino silver bromo-iodide emulsion. This emulsion is prepared by adding to  $\frac{1}{2}$  kg. of gelatino silver bromo-iodide emulsion (2% iodide) containing  $\frac{1}{6}$  mol of silver halide, 9 g. of a slightly alkaline alcoholic solution of 2-(1-phenyl-5-oxo-3-pyrazolinylimino)-3-carbethoxy-4-p-(1-n-hexadecyloxy)-phenyl-thiazoline, 6 g. of the mask compound 3-ethyl-2-benzothiazolone- $\beta$ -n-hexadecylsulfonyl hydrazone prepared according to our British patent specification No. 975,932 and having the following formula:



and dissolved by heating in a mixture of alcohol and water (1:3) with a little sodium hydroxide, acidifying with acetic acid to pH 6, and adding the usual additives such as hardeners, wetting agents, stabilizers and the necessary quantity of distilled water to obtain 1 kg. of flowable emulsion. The light sensitive multilayer photographic material is exposed through a grey-wedge, developed and further treated as described in Example 1. In the red-sensitive emulsion layer in addition to a cyan image also an orange to yellow dye mask image is formed, with a gradation opposed to that of the cyan image, and which compensates the side-absorptions of the cyan image in the blue as well as in the green region of the spectrum. In the green-sensitive emulsion layer in addition to a magenta dye image also a yellow dye mask image is formed, with a gradation opposed to that of the magenta image, and which reduces the disturbing influence of the side-absorptions in the formed magenta image.

## EXAMPLE 11

To  $\frac{1}{2}$  kg. of a red-sensitive bromo-iodide emulsion (3% of iodide) containing  $\frac{1}{6}$  mol of silver halide are added: (1) 10 g. of N-(6'-n-hexadecylsulfonyl-phenyl)-1-hydroxy-2-naphthoic acid amide-3'-sodium sulfonate dissolved in a mixture of 193 cm.<sup>3</sup> of water and 7 cm.<sup>3</sup>

of aqueous 2 N sodium hydroxide, and (2) 5 g. of the mask compound prepared according to Preparation 12, dissolved in a mixture of 37.5 cm.<sup>3</sup> of water and 12.5 cm.<sup>3</sup> N sodium hydroxide. After acidification with acetic acid to pH 6, the usual additives such as hardeners, wetting agents and stabilizers and the necessary quantity of distilled water are added to the emulsion in order to obtain 1 kg. of flowable emulsion. The emulsion is coated on a suitable support and dried. After exposure through a grey-wedge with a constant 0.15, the photographic material composed in this way is developed and further treated as in Example 1. In the exposed and processed strip, in addition to a cyan image also an orange mask image is formed, with a gradation opposed to that of the cyan image, and which compensates the side-absorptions of the cyan image in the blue as well as in the green region of the spectrum.

We claim:

1. In a method of forming a color corrected image in a photographic element having at least one silver halide emulsion layer containing a color coupler for magenta which is reactive with the oxidation product of an aromatic amino developing agent to form by color development a magenta primary dye image which absorbs a major proportion of light in one region of the visible spectrum, and undesirably absorbs a minor proportion of light in at least one other region of the visible spectrum, in which method said element is exposed to said image to be photographed, developed with said developing agent and thereafter treated with an oxidizing solution, the improvement wherein said element has present therein a mask-forming compound having the formula:



wherein

R<sub>1</sub> is a member of the group consisting of a hydrogen atom and an acyl radical,

R<sub>2</sub> is a member of the group consisting of a hydrogen atom, an amino radical, an alkyl radical, an alkylene radical, an aryl radical, and a heterocyclic radical,

Y represents the non-metallic atoms necessary to complete a nitrogen-containing heterocyclic nucleus, and

X is a member of the group consisting of an hydroxyl radical, an amino radical, an aliphatic hydrocarbon radical, an aryl radical, and a heterocyclic radical;

whereby the residual color coupler oxidatively couples with said mask-forming compound to form a secondary dye image having a gradation opposite to that of said magenta primary dye image, said secondary image absorbing regions but transmitting substantially all the light in said major absorption region.

2. The method of claim 1 wherein said color coupler for magenta is a member of the group consisting of the indazolone and pyrazolone color couplers.

3. The method of claim 1 wherein said oxidizing solution is a photographic bleaching bath.

4. The method of claim 1 wherein said mask-forming compound is present in at least said one emulsion layer.

5. The method of claim 2 wherein said mask-forming compound forms a yellow secondary dye image.

6. A color photographic element useful in the method of claim 1, said element having superposed silver halide emulsion layers sensitive to different regions of the visible spectrum, at least one of said layers containing a color coupler for magenta which is reactive with the oxidation product of an aromatic amino developing agent to form by color development a magenta primary dye image which absorbs a major proportion of light in one region of the spectrum, and undesirably absorbs a minor proportion of light in at least one other region of the

25

visible spectrum, such layer also containing a mask-forming compound of the formula:



wherein:

R<sub>1</sub> is a member of the group consisting of a hydrogen atom and an acyl radical,  
 Y represents the non-metallic atoms necessary to complete a nitrogen-containing heterocyclic nucleus,  
 R<sub>2</sub> is a member of the group consisting of a hydrogen atom, an amino radical, an alkyl radical, an alkylene radical, an aryl radical, and a heterocyclic radical, and  
 X is a member of the group consisting of an hydroxyl radical, an amino radical, an aliphatic hydrocarbon radical, an aryl radical, and a heterocyclic radical;

said color coupler for magenta also being reactive with the oxidation product of said mask-forming compound to form a secondary dye image having a gradation opposite to that of said magenta primary dye image, and absorbing light in at least one of said unwanted minor absorption regions but transmitting substantially all the light in said major absorption region.

7. The element of claim 6 wherein said color coupler for magenta is a member of the group consisting of the indazolone and pyrazolone color couplers.

8. In a method of forming a color corrected image in a photographic element having at least one silver halide emulsion layer containing a color coupler for cyan which is reactive with the oxidation product of an aromatic amino developing agent to form by color development a cyan primary dye image which absorbs a major proportion of light in one region of the visible spectrum, and undesirably absorbs a minor proportion of light in at least one other region of the visible spectrum, in which method said element is exposed to said image to be photographed, developed with said developing agent and thereafter treated with an oxidizing solution, the improvement wherein said element has present therein a mask-forming compound having a formula selected from the group consisting of:



and



wherein:

R<sub>1</sub> is a member of the group consisting of a hydrogen atom and an acyl radical,  
 R<sub>2</sub> is a member of the group consisting of a hydrogen atom, an amino radical, an alkyl radical, an alkylene radical, an aryl radical, and a heterocyclic radical,  
 R<sub>3</sub> and R<sub>4</sub> are each a member of the group consisting of a hydrogen atom, an alkyl radical, and an aryl radical,  
 Y represents the non-metallic atoms necessary to complete a nitrogen-containing heterocyclic nucleus, and  
 X is a member of the group consisting of an hydroxyl radical, an amino radical, an aliphatic hydrogen radical, an aryl radical, and a heterocyclic radical;  
 whereby the residual color coupler oxidatively couples with said mask-forming compound to form a secondary dye image having a gradation opposite to that of said cyan primary dye image, said secondary image absorbing light in at least one of said undesirable minor absorption regions but transmitting substantially all the light in said major absorption region.

9. The method of claim 8 wherein said color coupler

26

for cyan is a member of the group consisting of the phenol and naphthol color couplers.

10. The method of claim 9 wherein said color coupler has the formula:



wherein:

X<sub>2</sub> is a radical of the group consisting of —O—, —S—, —NHCO—, —CONH—, —SO<sub>2</sub>NH—, —NHSO<sub>2</sub>—, —N-alkyl

and —SO<sub>2</sub>—,

Z is a member of the group consisting of a hydrogen atom and a halogen atom,

D is an aliphatic radical comprising a linear chain of 5-20 carbon atoms, and

M is a member of the group consisting of a hydrogen atom, an alkali atom, and an ammonium group.

25 11. The method of claim 8 wherein said oxidizing bath is a photographic bleaching bath.

12. The method of claim 8 wherein said mask-forming compound is present in the same emulsion layer containing said color coupler.

30 13. The method of claim 9 wherein said mask-forming compound forms a yellow-to-magenta secondary dye image.

14. A color photographic element useful in the method of claim 8, said element having superposed silver halide emulsion layers sensitive to different regions of the visible spectrum, at least one of said layers containing a color coupler for cyan which is reactive with the oxidation product of an aromatic amino developing agent to form

35 by color development a cyan primary dye image which absorbs a major proportion of light in one region of the spectrum, and undesirably absorbs a minor proportion of light in at least one other region of the visible spectrum, such layer also containing a mask-forming compound of a formula selected from the group consisting of:

45



50 and



55 wherein:

R<sub>1</sub> is a member of the group consisting of a hydrogen atom and an acyl radical,

Y represents the non-metallic atoms necessary to complete a nitrogen-containing heterocyclic nucleus,

R<sub>2</sub> is a member of the group consisting of a hydrogen atom, an amino radical, an alkyl radical, an alkylene radical, an aryl radical, and a heterocyclic radical,

60 R<sub>3</sub> and R<sub>4</sub> are each selected from the group consisting of a hydrogen atom, an alkyl radical, and an aryl radical, and

X is a member of the group consisting of an hydroxyl radical, an amino radical, an aliphatic hydrogen radical, an aryl radical, and a heterocyclic radical;

65 70 said color coupler for magenta also being reactive with the oxidation product of said mask-forming compound to form a secondary dye image having a gradation opposite to that of said cyan primary dye image, and absorbing light in at least one of said unwanted minor absorption

75

regions but transmitting substantially all the light in said major absorption region.

15. The element of claim 14 wherein said color coupler for cyan is a naphthol color coupler having the formula:



5

10

15

wherein:

$X_2$  is a radical of the group consisting of  $-\text{O}-$ ,  $-\text{S}-$ ,  $-\text{NHCO}-$ ,  $-\text{CONH}-$ ,  $-\text{SO}_2\text{NH}-$ ,  $-\text{NHSO}_2-$ ,  $-\text{N-alkyl}$

and  $-\text{SO}_2-$ ,

$Z$  is a member of the group consisting of a hydrogen atom and a halogen atom,

$D$  is an aliphatic radical comprising a linear chain of 5-20 carbon atoms, and

$M$  is a member of the group consisting of a hydrogen atom, an alkali atom, and an ammonium group.

References Cited by the Examiner

UNITED STATES PATENTS

|           |         |                  |       |         |
|-----------|---------|------------------|-------|---------|
| 2,498,418 | 2/1950  | Hanford          | ----- | 96-55   |
| 2,518,739 | 8/1950  | Young            | ----- | 96-55   |
| 2,823,998 | 2/1958  | Jennen           | ----- | 96-100  |
| 2,994,607 | 8/1961  | Loffler et al.   | ----- | 96-9    |
| 3,012,884 | 12/1961 | De Ramaix et al. | ----- | 96-9    |
| 3,013,879 | 12/1961 | De Ramaix        | ----- | 96-55 X |
| 3,047,385 | 7/1962  | De Ramaix et al. | ----- | 96-9    |

FOREIGN PATENTS

|         |         |                |
|---------|---------|----------------|
| 685,061 | 12/1952 | Great Britain. |
| 790,327 | 2/1958  | Great Britain. |

NORMAN G. TORCHIN, Primary Examiner.

20 HAROLD N. BURSTEIN, Examiner.

R. A. BURROUGHS, J. T. BROWN,  
Assistant Examiners.